# EUROPEAN PATENT SPECIFICATION

(11) **EP 3 405 613 B1**
(45) Date of publication and mention of the grant of the patent: **22.01.2020**
(21) Application number: 17702618.4
(22) Date of filing: 01.02.2017
(51) Int. Cl.: D21H 19/66, D21H 19/82, D21H 19/40, D21H 17/67, D21H 21/18

(54) **PEARLESCENT METALLIC EFFECT PAPER MATERIAL WITH HIGH LIGHTFASTNESS AND RELATED MANUFACTURING METHOD**
PAPIERMATERIAL MIT PERLGLÄNZENDEM METALLEFFEKT UND HOHER LICHTBESTÄNDIGKEIT SOWIE ZUGEHÖRIGES HERSTELLUNGSVERFAHREN
MATÉRIAU EN PAPIER À EFFET MÉTALLIQUE NACRÉ PRÉSENTANT UNE RÉSISTANCE ÉLEVÉE À LA LUMIÈRE ET PROCÉDÉ DE FABRICATION ASSOCIÉ

(30) Priority: 01.02.2016 IT UB20160512
(43) Date of publication of application: 28.11.2018
(73) Proprietor: Gruppo Cordenons S.p.A., 20145 Milano (IT)
(72) Inventor: MONACELLI, Luca, 33084 Cordenons (Pordenone) (IT); GILBERTI, Ferruccio, Beniamino, 20121 Milano (IT)
(74) Representative: Rapisardi, Mariacristina
(86) International application number: PCT/EP2017/052094
(87) International publication number: WO 2017/134071

(56) References cited:
- EP-A1- 2 520 709
- WO-A1-02/12621
- WO-A1-99/16708
- WO-A1-2004/007215
- WO-A1-2004/099500
- WO-A1-2014/198780
- US-A- 5 571 557
- US-A1- 2013 052 243

## Description

The present invention refers to a paper material (paper/card) and to the relative manufacturing method.

In the paper sector, there is a constant search for new types of paper having particular characteristics and finishes, especially papers designed for packing, packaging, realizing illustrative material, quality printing, etcetera.

WO2014/198780 A1 discloses a paper material (paper/pasteboard) having holographic and pearlescent metallic effects and the manufacturing process thereof; EP2520709A1 discloses sand effect paper material and corresponding manufacturing method; WO2004/099500A1 refers to a method for producing coated paper with pearlescent effect; WO02/12621A1 teaches a process for the preparation of paper having a special appearance; US5571557A relates to faux glass etch product and process of preparing the same; WO2004007215A1 refers to papers for use in decorative laminates and methods of making the same; US2013052243A1 teaches a composite material of inorganic non-metallic mineral loaded with titania layer, preparation process and use thereof, and WO9916708A1 discloses colloidal borosilicates and their use in the production of paper.

However, it is not uncommon that the achievement of special effects is detrimental to other characteristics of the paper, such as printability.

A technical task of the present invention is to provide a paper material that has a different optical effect from conventional paper materials, while also being printable with high printing quality.

This technical task is solved by a paper material comprising a base support, made up of a mixture of cellulose fibres containing at least one polymeric substance, which is adapted to give the mixture of fibres mechanical strength, and an inorganic filler, said base support having at least one surface treated with at least one surface adhesive and at least one coating applied on said treated surface, characterized in that said coating comprises at least pearlescent pigments of high lightfastness, said pearlescent pigments being transparent borosilicates or aluminosilicates coated with metal oxides..

The present invention also discloses a method for manufacturing the paper material, comprising the steps of:
- preparing an aqueous pulp of cellulose fibres, containing at least one polymeric substance adapted to give the mixture of fibres mechanical strength, and an inorganic filler;
- removing water from the pulp so as to form a base support of the paper material;
- treating at least one surface of the base support with at least one surface adhesive;
- performing a smoothing process on the treated surface of the base support;
- applying a coating comprising at least pearlescent pigments of high lightfastness to the smoothed treated surface, said pearlescent pigments being transparent borosilicates or aluminosilicates coated with metal oxides.

In a preferred embodiment the pearlescent pigments are micas.

In a preferred embodiment the pearlescent pigments are transparent borosilicates or aluminosilicates coated with metal oxides such as iron oxides, titanium oxides or tin oxides.

In a preferred embodiment the pearlescent pigments are of various colours, particle sizes and shapes.

In a preferred embodiment the coating comprises one or more binder polymers and/or waxes, in a mixture with said pearlescent pigments.

In a preferred embodiment the coating comprises one or more binder polymers and/or waxes, in a mixture with said pearlescent pigments and with magnetic or diamagnetic metallic pigments.

In a preferred embodiment the metallic pigments are of various colours, particle sizes and shapes.

In a preferred embodiment the metallic effect pigments of the coating are those normally used for exterior grade paint.

Therefore the coating contains pearlescent pigments and can optionally contain metallic pigments as well as the pearlescent pigments.

Furthermore, the coating may also contain organic and inorganic pigments in addition to the pearlescent pigments and the metallic pigments.

There may also be organic or inorganic pigments contained in the base support which may be coloured.

The invention therefore provides a pearlescent paper material (paper/card) of high lightfastness, thanks to a specially designed pulp and a specific surface coating treatment.

The paper material of the invention also proves to be perfectly printable with high printing quality and makes it possible to achieve particular graphic effects that are difficult to achieve with conventional coated papers.

In detail, the paper material of the invention comprises a base support made up of a mixture of cellulosic fibres and it contains at least one polymeric substance, adapted to give the mixture of fibres mechanical strength (when dry or wet), and an inorganic filler, adapted to give the material good machinability characteristics.

The base support has at least one surface (face) treated with at least one surface adhesive to which a coating is applied, so that, due to the combined effect of the composition of the base support and the surface treatment, the paper material has a pearlescent effect with various colours. Clearly, both faces of the base support may be treated in the same way.

Preferably, the polymeric substance included in the base support comprises one or more colophony-based and/or alkyl-ketene-dimer-based and/or acetylsuccinic-acid-based and/or epochlorohydrin-based resins, and/or modified starches; and the inorganic filler is a mineral filler comprising one or more substances selected from the group constituted by carbonates, kaolins, talc and mixtures thereof.

The surface adhesive is for example an adhesive based on starch and/or polyvinyl alcohol- and/or acrylic-, polyurethane- and/or styrene-butadiene-based polymers.

As mentioned, the paper material according to the invention is provided with a coating, applied on the treated surface and clearly, the paper material may have both surfaces treated and provided with a coating.

In particular, the coating is formed by one or more binder polymers (e.g. polyurethane- and/or silicone-, and/or acrylic-, styrene-butadiene-, polyvinyl acetate-, polyvinyl alcohol-based polymers and the like) and/or waxes, in a mixture with dyes and pigments, e.g. pearlescent pigments of various colours, particle sizes and shapes with the characteristic of being stable to the exposure of the UV component of sunlight.

The quantity of polymer per face is preferably comprised between 5% by weight and 100% by weight with respect to the pigments; the paper basis weight of the paper material is comprised between about 90 and about 450 g/m²; the quantity of coating spread onto each face is comprised between about 5 and about 20 g/m².

The coating may be coloured and/or spread onto a coloured base support; preferably, coloured pastes and organic or inorganic pigments are used.

In accordance with a further aspect of the present invention, the paper material described hereinabove is realized using the following method.

The base support is realized first, using a substantially known paper-forming technique, for example on a continuous machine for manufacturing paper.

In essence, an aqueous pulp comprising a mixture of cellulose fibres and containing the polymeric substance (colophony-based and/or alkyl-ketene-dimer-based and/or acetylsuccinic-acid-based and/or epochlorohydrin-based resins, and/or modified starches) and the inorganic filler (carbonates, kaolins, talc, etcetera) is prepared.

Subsequently, water is removed from the pulp so as to form a base support of the paper material.

This is followed by a step of surface treatment of one or both faces of the base support with an aqueous solution of surface adhesive, for example made up of a 10% by weight aqueous solution of starch, and/or 5% by weight of acrylic adhesive, or similar adhesives.

After the surface treatment with adhesive, the method then comprises a smoothing step of the base support, wherein the base support is smoothed up to Bendtsen ISO 2494 roughness values of less than approximately 450 ml/min., preferably of less than approximately 400 ml/min. and approximately around 350 ml/min, followed by an application step of the coating previously described.

Preferably, the application of the coating takes place by spreading with an air knife or a smoothing blade, roto-offset, rotographic and flexographic techniques.

This is followed by step of drying the coating, carried out in an infrared and/or hot-air oven at a temperature within the range of 100°C approximately to 180°C approximately and with an oven time ranging between 0.5 and 4 minutes.

Lastly, the method comprises a step of mechanically treating the surface provided with the coating, particularly a smoothing and/or an embossing step.

It remains understood that modifications and variants that are not beyond the scope of the invention as defined in the appended claims, may be made concerning the paper material and the relative manufacturing method disclosed and illustrated herein.

## Claims

1. A paper material comprising a base support, made up of a mixture of cellulose fibers containing at least one polymeric substance, which is adapted to give the mixture of fibers mechanical strength, and an inorganic filler, said base support having at least one surface treated with at least one surface adhesive and at least one coating applied on said treated surface, **characterized in that** said coating comprises at least pearlescent pigments of high lightfastness, said pearlescent pigments being transparent borosilicates or aluminosilicates coated with metal oxides.

2. The paper material according to claim 1, **characterized in that** said pearlescent pigments are of various colors, particle sizes and shapes.

3. The paper material according to claim 1, **characterized in that** said coating comprises one or more binder polymers and/or waxes, in a mixture with said pearlescent pigments.

4. The paper material according to claim 1, **characterized in that** said coating comprises one or more binder polymers and/or waxes, in a mixture with said pearlescent pigments and with magnetic or diamagnetic metallic pigments.

5. The paper material according to any one of the preceding claims, **characterized in that** the polymeric substance included in the base support comprises one or more colophony-based and/or alkyl-ketene-dimer-based and/or acetylsuccinic-acid-based and/or epochlorohydrin-based resins, and/or modified starches.

6. The paper material according to any one of the preceding claims, **characterized in that** the inorganic filler is a mineral filler and it comprises one or more substances selected from the group constituted by carbonates, kaolins, talc and mixtures thereof

7. The paper material according to any one of the preceding claims, **characterized in that** the surface adhesive is an adhesive based on starch and/or polyvinyl alcohol and/or acrylic, polyurethane and/or styrene-butadiene polymers.

8. The paper material according to any one of claims 3 to 6 **characterized in that** the binder polymers comprise polyurethane-, acrylic-, polyvinyl alcohol-, styrene-butadiene and/or silicone-based polymers.

9. A method for manufacturing a paper material, comprising the steps of:
- preparing an aqueous pulp of cellulose fibers, containing at least one polymeric substance adapted to give the mixture of fibers mechanical strength, and an inorganic filler;
- removing water from the pulp so as to form a base support of the paper material;
- treating at least one surface of the base support with at least one surface adhesive;
- performing a smoothing process on the treated surface of the base support;
- applying a coating comprising at least pearlescent pigments of high lightfastness to the smoothed treated surface, said pearlescent pigments being transparent borosilicates or aluminosilicates coated with metal oxides .

10. The method according to the preceding claim, **characterized in that** the treated surface is smoothed up to Bendtsen ISO 2494 roughness values of less than approximately 450 ml/min., preferably of less than approximately 400 ml/min. and approximately around 350 ml/min.

11. The method according to claim 9 or 10, **characterized in that** the coating applied to the treated surface comprises, in a mixture, said pearlescent pigments, magnetic or diamagnetic metallic pigments, and one or more binder polymers and/or waxes.

12. The method according to any one of claims 9 to 11, **characterized in that** the step of applying the coating takes place by spreading with an air knife or a smoothing blade.

13. The method according to any one of claims 9 to 12, **characterized in that** it comprises a step of drying the coating, carried out in an infrared and/or hot-air oven at a temperature within the range of 100°C approximately to 180°C approximately and with an oven time ranging between 0.5 and 4 minutes.

14. The method according to claim 13, **characterized in that** after drying the coating, a step of mechanically treating the surface provided with the coating is performed, particularly a smoothing step and/or an embossing step.

## Patentansprüche

1. Papiermaterial, umfassend einen Grundträger, der aus einer Mischung aus Cellulosefasern besteht, die mindestens eine polymere Substanz, die geeignet ist, der Mischung aus Fasern mechanische Festigkeit zu verleihen, und einen anorganischen Füllstoff enthält, wobei der Grundträger mindestens eine Oberfläche aufweist, die mit mindestens einem Oberflächenklebstoff und mindestens einer Beschichtung, die auf die behandelte Oberfläche aufgebracht sind, behandelt ist, **dadurch gekennzeichnet, dass** die Beschichtung mindestens perlglänzende Pigmente mit hoher Lichtbeständigkeit umfasst, wobei die perlglänzenden Pigmente mit Metalloxiden beschichtete transparente Borosilikate oder Aluminosilikate sind.

2. Papiermaterial nach Anspruch 1, **dadurch gekennzeichnet, dass** die perlglänzenden Pigmente verschiedene Farben, Partikelgrößen und Formen aufweisen.

3. Papiermaterial nach Anspruch 1, **dadurch gekennzeichnet, dass** die Beschichtung ein oder mehrere Bindemittelpolymere und/oder Wachse in einer Mischung mit den perlglänzenden Pigmenten umfasst.

4. Papiermaterial nach Anspruch 1, **dadurch gekennzeichnet, dass** die Beschichtung ein oder mehrere Bindemittelpolymere und/oder Wachse in einer Mischung mit den perlglänzenden Pigmenten und mit magnetischen oder diamagnetischen Metallpigmenten umfasst.

5. Papiermaterial nach einem der vorhergehenden Ansprüche, **dadurch gekennzeichnet, dass** die im Grundträger eingeschlossene polymere Substanz ein oder mehrere Harze auf Kolophoniumbasis und/oder Alkylketendimerbasis und/oder Acetylbernsteinsäurebasis und/oder auf Epochlorhydrinbasis und/oder modifizierte Stärken umfasst.

6. Papiermaterial nach einem der vorhergehenden Ansprüche, **dadurch gekennzeichnet, dass** der anorganische Füllstoff ein mineralischer Füllstoff ist und es eine oder mehrere Substanzen umfasst, die aus der Gruppe ausgewählt sind, die aus Carbonaten, Kaolinen, Talk und Mischungen davon besteht.

7. Papiermaterial nach einem der vorhergehenden Ansprüche, **dadurch gekennzeichnet, dass** der Oberflächenklebstoff ein Klebstoff auf Basis von Stärke und/oder Polyvinylalkohol und/oder Acryl-, Polyurethan- und/oder Styrol-Butadien-Polymeren ist.

8. Papiermaterial nach einem der Ansprüche 3 bis 6, **dadurch gekennzeichnet, dass** die Bindemittelpolymere Polymere auf Polyurethan-, Acryl-, Polyvinylalkohol-, Styrol-Butadien- und/oder Silikonbasis umfassen.

9. Verfahren zur Herstellung eines Papiermaterials, umfassend die Schritte:
- Herstellen einer wässrigen Pulpe aus Cellulosefasern, enthaltend mindestens eine polymere Substanz, die geeignet ist, der Mischung aus Fasern mechanische Festigkeit zu verleihen, und einen anorganischen Füllstoff;
- Entfernen von Wasser aus der Pulpe, um einen Grundträger des Papiermaterials zu bilden;
- Behandeln mindestens einer Oberfläche des Grundträgers mit mindestens einem Oberflächenklebstoff;
- Durchführen eines Glättungsprozesses auf der behandelten Oberfläche des Grundträgers;
- Aufbringen einer Beschichtung umfassend mindestens perlglänzende Pigmente mit hoher Lichtbeständigkeit auf die geglättete behandelte Oberfläche, wobei die perlglänzenden Pigmente mit Metalloxiden beschichtete transparente Borsilikate oder Aluminosilikate sind.

10. Verfahren nach dem vorhergehenden Anspruch, **dadurch gekennzeichnet, dass** die behandelte Oberfläche auf Rauheitswerte nach Bendtsen ISO 2494 von weniger als etwa 450 ml/min., vorzugsweise von weniger als etwa 400 ml/min. und etwa um 350 ml/min. geglättet wird.

11. Verfahren nach Anspruch 9 oder 10, **dadurch gekennzeichnet, dass** die auf die behandelte Oberfläche aufgebrachte Beschichtung in einer Mischung die perlglänzenden Pigmente, die magnetischen oder diamagnetischen Metallpigmente und ein oder mehrere Bindemittelpolymere und/oder Wachse umfasst.

12. Verfahren nach einem der Ansprüche 9 bis 11, **dadurch gekennzeichnet, dass** der Schritt zum Aufbringen der Beschichtung durch Verteilen mit einem Luftmesser oder einer Glättungsklinge erfolgt.

13. Verfahren nach einem der Ansprüche 9 bis 12, **dadurch gekennzeichnet, dass** es einen Schritt zum Trocknen der Beschichtung umfasst, der in einem Infrarot- und/oder Heißluftofen bei einer Temperatur im Bereich von etwa 100 °C bis etwa 180 °C und mit einer Ofenzeit zwischen 0,5 und 4 Minuten durchgeführt wird.

14. Verfahren nach Anspruch 13, **dadurch gekennzeichnet, dass** nach dem Trocknen der Beschichtung ein Schritt zum mechanischen Behandeln der mit der Beschichtung versehenen Oberfläche durchgeführt wird, insbesondere ein Glättungsschritt und/oder ein Prägeschritt.

## Revendications

1. Matériau en papier comprenant un support de base composé d'un mélange de fibres de cellulose contenant au moins une substance polymère pouvant conférer une force mécanique au mélange de fibres, et une charge inorganique, ledit support de base ayant au moins une surface traitée avec au moins un adhésif de surface et au moins un couchage appliqué sur ladite surface traitée, **caractérisé en ce que** ledit couchage comprend au moins des pigments nacrés très résistants à la lumière, lesdits pigments nacrés étant des borosilicates ou des aluminosilicates transparents avec couche d'oxydes métalliques.

2. Matériau en papier selon la revendication 1, **caractérisé en ce que** lesdits pigments nacrés sont de plusieurs couleurs, granulométries et formes.

3. Matériau en papier selon la revendication 1, **caractérisé en ce que** ledit couchage comprend un ou plusieurs liants polymères et/ou cires, en mélange avec lesdits pigments nacrés.

4. Matériau en papier selon la revendication 1, **caractérisé en ce que** ledit couchage comprend un ou plusieurs liants polymères et/ou cires, en mélange avec lesdits pigments nacrés et avec des pigments métalliques magnétiques ou diamagnétiques.

5. Matériau en papier selon l'une quelconque des revendications précédentes, **caractérisé en ce que** la substance polymère incluse dans le support de base comprend une ou plusieurs résines à base de colophane et/ou de dimère d'alkylcétène et/ou d'acide acétylsuccinique et/ou d'épichlorhydrine, et/ou d'amidons modifiés.

6. Matériau en papier selon l'une quelconque des revendications précédentes, **caractérisé en ce que** la charge inorganique est une charge minérale et comprend une ou plusieurs substances sélectionnées dans le groupe composé de carbonates, kaolins, talc et leurs mélanges.

7. Matériau en papier selon l'une quelconque des revendications précédentes, **caractérisé en ce que** l'adhésif de surface est un adhésif à base d'amidon et/ou d'alcool polyvinylique et/ou de polymères d'acrylique, de polyuréthane et/ou de styrène-butadiène.

8. Matériau en papier selon l'une quelconque des revendications de 3 à 6, **caractérisé en ce que** les liants polymères comprennent des polymères à base de polyuréthane, d'acrylique, d'alcool polyvinylique, de styrène-butadiène et/ou de silicone.

9. Procédé de fabrication d'un matériau en papier, comprenant les étapes de :
- préparer une pâte aqueuse de fibres de cellulose contenant au moins une substance polymère pouvant conférer une force mécanique au mélange de fibres, et une charge inorganique ;
- retirer l'eau de la pâte de sorte à former un support de base du matériau en papier ;
- traiter au moins une surface du support de base avec au moins un adhésif de surface ;
- exécuter un lissage sur la surface traitée du support de base ;
- appliquer sur la surface traitée lissée un couchage comprenant au moins des pigments nacrés très résistants à la lumière, lesdits pigments nacrés étant des borosilicates ou des aluminosilicates transparents avec couche d'oxydes métalliques.

10. Procédé selon la revendication précédente, **caractérisé en ce que** la surface traitée est lissée à des valeurs de rugosité Bendtsen ISO 2494 de moins de 450 ml/min approximativement, de préférence de moins de 400 ml/min approximativement, et aux alentours de 350 ml/min.

11. Procédé selon la revendication 9 ou 10, **caractérisé en ce que** le couchage appliqué sur la surface traitée comprend, en mélange, lesdits pigments nacrés, lesdits pigments métalliques magnétiques ou diamagnétiques, et un ou plusieurs liants polymères et/ou cires.

12. Procédé selon l'une quelconque des revendications de 9 à 11, **caractérisé en ce que** l'étape d'application du couchage se fait par pulvérisation avec une lame d'air ou avec une lame de lissage.

13. Procédé selon l'une quelconque des revendications de 9 à 12, **caractérisé en ce qu'**il comprend une étape de séchage du couchage, réalisée dans un four à infrarouges et/ou dans un four à air chaud à une température comprise approximativement entre 100 et 180 °C pendant une durée comprise entre 0,5 et 4 minutes.

14. Procédé selon la revendication 13, **caractérisé en ce qu'**après le séchage du couchage, la surface pourvue du couchage est traitée mécaniquement, en particulier une étape de lissage et/ou une étape de gaufrage.
